

# UNITED STATES PATENT OFFICE.

HENRY HOWARD, OF BOSTON, MASSACHUSETTS.

## METHOD OF TREATING IRON OR STEEL ARTICLES.

949,575.

Specification of Letters Patent. Patented Feb. 15, 1910.

No Drawing.

Application filed November 16, 1909. Serial No. 528,369.

To all whom it may concern:

Be it known that I, HENRY HOWARD, a citizen of the United States, residing at Boston, in the county of Suffolk and State 5 of Massachusetts, have invented certain new and useful Improvements in Methods of Treating Iron or Steel Articles, of which the following is a specification.

This invention relates to the preparation 10 of sheets or other forms of iron and steel for tinning or galvanizing.

It is well known that tinned plates are very frequently imperfect by reason of the presence of minute uncovered areas, perforations, or so-called "pin holes" in the coating metal, such imperfections being highly detrimental by reason of the tendency of the coated metal to become corroded or pitted at these points or areas. While all surfaces 20 of iron or steel which have been thoroughly cleaned and freed from grease or oxid are very susceptible to oxidation or corrosion, such imperfections are particularly liable to occur in plates which have been subjected to an acid pickling process; and their presence may in this case be partly or wholly attributed to the persistence in the metal 25 to be coated of acid conditions arising from the baths employed for the removal of the scale.

The object of the present invention is the provision of a more rapid and effective method of securing complete and certain elimination of such acid conditions, and in 30 general a more complete protection of coated surfaces from corrosive influences, than is practicable by known methods, for example in the case of pickled plates, by washing with alkaline solutions.

According to the preferred embodiment of the invention, the iron or steel articles are first freed from scale by the usual methods, as by immersion for a suitable time in an acid pickling bath. The articles are then 40 immersed, preferably after a brief washing or rinsing with water or a suitable alkaline solution, in an alkaline electrolyte, being connected therein as the cathode. As electrolytes, solutions containing a carbonate or

hydroxid of an alkali are most suitable. 50 An electric current is passed to the sheet or other article as cathode, resulting in the deposition or separation of the alkali metal, and by secondary reaction of this metal with the water of the solution, in an evolution of 55 hydrogen at the surface of the metal. By this procedure the cleaned surfaces are rendered far less liable to corrosion, any residual acid conditions are quickly eliminated, and the metal may immediately receive a coating of tin or zinc by immersion in the molten metal in the usual way.

I am aware that it has been proposed to clean metal sheets, preliminary to coating them, by connecting them as cathode in acid 60 or alkaline solutions, but in such cases the purpose has been to utilize the evolved gas for the mechanical removal of scale, grease and the like, that is to say for cleaning the plates; whereas according to the present invention the electrolytic treatment is applied to sheets or articles which have already undergone a cleaning operation, and which by reason of their freedom from scale or 65 grease are highly susceptible to corrosion, the purpose of the treatment being to render the plates or articles less liable to subsequent pitting or corrosion and to secure in a rapid and certain manner the elimination of all 70 residual acid conditions and the provision of a surface which is capable of receiving, by the usual coating methods, a more perfect film of coating metal.

I claim:—

The method of preparing iron and steel 80 articles for tinning or galvanizing, which consists in subjecting the articles to an acid pickling process to remove the scale and thereafter passing an electric current to the cleaned articles connected as cathode in an 85 alkaline electrolyte.

In testimony whereof, I affix my signature in presence of two witnesses.

HENRY HOWARD.

Witnesses:

EVERETT EDWIN BRAINARD,  
HERBERT S. KIMBALL.